

Jan. 19, 1937.

F. R. SEAVEY

2,068,516

STRATIFIED PRIMER CHARGE

Filed July 14, 1933

Fig. 1.



Fig. 2.



Fig. 3.



Fig. 4.

Inventor:  
FREDERICK R. SEAVEY,  
305 John H. Brumaga,  
His Attorney.

## UNITED STATES PATENT OFFICE

2,068,516

## STRATIFIED PRIMER CHARGE

Frederick R. Seavey, Alton, Ill., assignor to  
 Western Cartridge Company, East Alton, Ill., a  
 corporation of Delaware

Application July 14, 1933, Serial No. 680,347

13 Claims. (Cl. 102—18)

This invention relates generally to primers, and particularly to a process of making primers for ammunition in which the necessary quantity of initiator is substantially reduced.

In primers of the type generally employed in small arms ammunition, and particularly with primers of the anvil type, it is apparent that only that portion of the initiator which is effective in initiating the ignition of the composition is that portion which is disposed so as to be acted upon by the detonating blow or initial action of the firing pin or striker blow transmitted through the metal of the primer cup, or in the case of primers of the stab-type (anvil-less) (open or metal foiled) to the initial action of the penetrating firing pin. For instance, with primers of the anvil type, it is apparent that the ignition of the priming mixture is initiated by the action of a relatively small volume of initiator which is disposed immediately adjacent the anvil point and the primer cup. It has been the general practice heretofore to incorporate an initiating ingredient throughout a priming mixture comprising other constituents, such as sensitizers, oxidizers and fuels, and to dispose such a mixture within a primer cup for action of a firing pin or anvil, but in view of the fact, however, that a relatively small quantity of initiator may be so placed that it will be acted upon by the detonating blow and will be capable of initiating the detonation, it is an object of the present invention to provide an arrangement of ingredients in a primer which will result in a substantial saving of the more expensive initiator.

The object of the present invention, generally stated, is to provide a primer in which the quantity of initiating ingredients employed is reduced to a minimum.

Another object of the invention is to provide a primer in which a highly sensitive mixture is exposed directly to the action of a detonating blow while a less sensitive mixture is disposed to be ignited by the initiator.

A further object of this invention is to provide a primer composed of increments of at least two priming mixtures, so disposed that the more sensitive increment is subjected to initiation by impact, the less sensitive increment ignited by the detonating or burning, or both, of the initiating mixture, and that the combined action of both will function the next unit in the ignition or explosive train of the article in which the primer may be used.

A further object of the invention is to provide

a primer in which the ingredients are so arranged that excessive pressures will be avoided, but proper ignition of the propellant charge accomplished.

Other objects will become apparent to those skilled in the art when the following description of several illustrative embodiments is read in connection with the accompanying drawing. It is to be understood, however, that the invention is not limited to the particular embodiments which are hereinafter specifically described for the purposes of illustration, but that the present invention is susceptible of use in primers generally and without regard to the particular ingredients which enter into the priming composition.

In the accompanying drawing:

Figure 1 is a sectional view showing one arrangement of primer strata in a typical anvil primer assembly.

Figure 2 is a similar view of another arrangement.

Figure 3 is a similar view of a further embodiment.

Figure 4 is a similar view of a still further embodiment.

In accordance with the present invention the sensitive ingredient of the priming composition is so located in the primer cup, and particularly with reference to the point of the anvil that the quantity of initiator necessary to properly prime the ammunition may be substantially reduced. The present invention contemplates that the initiating substance, whether used alone or mixed with other ordinary priming ingredients, be concentrated in a region adjacent the point of the anvil and in the bottom of the primer cup so as to receive the detonating blow. A relatively small quantity of initiator or composition containing the initiator is sufficient to ignite a fuel ingredient capable of producing suitable heat and flame. Accordingly the sensitive increment containing the initiator may be covered or surrounded by what will be referred to as a relatively insensitive increment which may contain suitable heat and flame producing ingredient. The secondary or insensitive increment may be of the same composition as the sensitive increment except that the initiating ingredients may be eliminated, or may be of entirely different composition depending upon the characteristics desired. The relatively sensitive and relatively insensitive increments or strata may be arranged in any number of various ways, and for the purpose of illustration will hereinafter be

described. It is a feature of particular advantage of the present invention, however, that the entire priming charges do not necessarily contain the highly sensitive, more costly initiating ingredient, but such of the initiating ingredient as is employed as disposed where its effect will be greatest. Likewise the use of customary abrasive sensitizers such as glass becomes unnecessary, except in that increment which is to respond to the detonating blow of the firing pin.

In view of the fact that the sensitivity of the secondary mixture to friction or impact, such as is produced by a detonating blow of a firing pin is immaterial, it is apparent that a sufficient quantity of suitable binder may be so incorporated with the fuel and oxidizing ingredients to render the mixture completely waterproof. Accordingly when the initiating mixture is covered with a layer of secondary mixture in which a waterproofing binder is incorporated in excess of the percentage of waterproofing binder incorporated in the sensitive mixture the whole will be rendered more waterproof without interfering with the sensitivity of the primer.

As used throughout this description the word "initiator" will be understood in its ordinary sense as contemplating the highly sensitive priming ingredients, such for instance as mercury fulminate, lead azide and the like. The word "oxidizer" will be understood in its ordinary sense as meaning such materials as potassium chlorate, barium nitrate, and the like. Likewise the word "fuel" is used in its ordinary sense in this art as contemplating readily combustible substances, such for instance as antimony sulphide, lead sulphocyanate, ferro silicon, aluminum, zirconium, nitrosoguanidine, guanidine picrate, and the like. The features of the present invention are applicable alike to the loading of either wet or dry mixtures although in the following descriptions there is described no specific embodiment in which the mixture is loaded dry.

A conventional battery cup assembly is illustrated in the drawing and may comprise a battery cup 1 receiving in one end thereof a priming cup 2 adapted to contain the priming composition and receive the detonating blow from the firing pin of a weapon. Disposed on the inside of the battery cup may be an anvil 3 having a point 4 extending into the region of the priming cup. In the end of the battery cup 1 which extends into the region of the propellant charge may be an opening 5 through which the flame may be propagated. If desired, a suitable covering, as for instance a piece of metal foil 6 may cover the opening 5. The primer assembly illustrated in the drawing and described above is illustrative of a conventional type, but it will be understood that the features of the present invention are not limited to use in connection with such assemblies but are applicable to primers generally.

As a specific illustration of such a primer, Figure 1 shows a stratified arrangement wherein a pellet 10 of an ordinary priming composition, such as one made up of a lead azide-zirconium-ferro silicon-barium nitrate-cellulose acetate mix is placed in the bottom of a primer cup and adjacent the point of anvil. Upon pellet 10 may be superimposed a layer 11 comprising a mixture of fuel and oxidizing agents with or without a suitable waterproofing binder. As an example of such a mixture would be one containing lead sulphocyanate, ferro silicon, barium nitrate and cellulose acetate. In fact the layer

11 may be of the same composition as pellet 10, but without the initiator.

As illustrated in Figure 2 of the drawing the secondary or insensitive increment is in the form of an annular ring 12 which may be formed in the primer cup as shown. In the central opening of the ring 12 may be placed a plug 13 of composition containing the initiator which has been heretofore described as a sensitive or priming increment. As clearly shown in Figure 2 the point 4 of the anvil extends into the sensitive mixture 13. It may be advantageous to incorporate a waterproofing binder in the composition of plug 13. The use of 1-2½% ester gum in either or both increments improves the stability and dependability of the primer without substantial reduction of the sensitivity.

A further illustrative embodiment is shown in Figure 3 and may be charged as follows; a suitable initiator, such as for instance lead azide, and, if it is desired, a suitable sensitizer such as glass, may be suspended in a suitable vehicle, such as for instance a solution of gum arabic and dichlorethyl ether, and as many drops of the suspension as is desired dropped directly into position in the primer cup and preferably adjacent the point of the anvil as shown at 14. By thus forming a suspension of the initiating mixture it may be readily placed in the desired position in the cup as by dropping. Although the presence of such a binding material as gum arabic or Canada balsam is not to be regarded as necessary, such binders, nevertheless, facilitate in the handling of the materials and maintain the same in position in the primer cup during the subsequent loading. After the initiating mixture has been thus placed in position a suitable secondary mixture 15 preferably containing a fuel ingredient and an oxidizing agent may be placed in position in the cup and covering the initiating mixture.

As illustrative of a slightly modified procedure, reference being had to Figure 4, the primer cup 2 may be first provided with a small amount of finely powdered glass 17 which may be suitably fixed therein, as for instance by cementing to the center of the cup, and in position which will be adjacent the point of the anvil 3. Over the glass may then be deposited a drop of initiator 18, such for instance as lead azide in suspension and this then covered with a secondary mixture 19 as described above.

From the foregoing description it is apparent that when various ingredients of a priming mixture are arranged in strata or layers in a primer cup with a small quantity of initiator in a position for direct action of a detonating blow, such as for instance immediately adjacent the point of the anvil, a substantial economy of the more highly priced initiating ingredients is rendered possible by reduction in the necessary amount thereof. By thus reducing the amount of initiator employed excessive pressures in the primer cup, or shall, which have heretofore been experienced with violent initiators may be avoided. At the same time, however, proper ignition of the propellant charge may be assured by increasing the amount of heat or flame producing ingredients without affecting the sensitivity.

It is apparent that by thus arranging the various ingredients of a priming mixture in the strata, or increments, it becomes possible to employ materials in the priming mixture which, although useful together have heretofore been re-

garded as incompatible in the same mixture because of the danger of reaction. By using immiscible binders and solvents in the different strata, the incompatible ingredients will be maintained in segregation without danger of reaction. Furthermore when a secondary charge, containing for instance a fuel and oxidizer, is superimposed upon or surrounds an initiating mixture in the manner hereinbefore described, it is apparent that complete waterproofing of the entire priming mixture is rendered readily possible. This has heretofore been generally regarded as impossible, particularly for the reason that waterproofing agents generally operate as deterrents and thus generally decrease the sensitivity of the initiating ingredients to which they might be exposed. With an arrangement such as hereinbefore described, it is apparent, however, that the use of higher percentages of waterproofing material may be confined to the secondary charge which preferably contains no initiating substances and accordingly the sensitivity of the primer will be unimpaired by the use of waterproofing binders. Moreover, in view of the high percentage of initiator in the sensitive increment the waterproofing material may be incorporated in it also without seriously affecting its operation.

From the foregoing description it is apparent that many modifications of the arrangement of the priming ingredients in a priming cup hereinbefore described will present themselves to those skilled in the art without departing from the spirit of the invention. It is to be specifically understood, therefore, that the invention is not limited to the specific details hereinbefore set forth, and that such individual features and sub-combinations of features as do not depart from the spirit of this invention are, although not specifically described herein, contemplated by and within the scope of the appended claims.

Having thus described the invention what is claimed is:

1. In a primer having an anvil, the combination comprising, a relatively small quantity of sensitive priming mixture containing sufficient of an initiator to produce desired sensitivity characteristics for the primer disposed adjacent the anvil point, and a less sensitive layer containing sufficient of a fuel and an oxidizing agent to produce the heat, flame and gas producing characteristics for the primer superimposed upon the sensitive mixture.

2. A primer comprising, a plug of sensitive composition containing an initiator, and relatively insensitive composition containing an oxidizing agent arranged as a ring around the plug.

3. A charge for an anvil primer comprising, a plug of sensitive primer composition adjacent the point of the anvil, and a ring of relatively insensitive but explosive composition surrounding the plug in adjacent relation.

4. A charge for an anvil primer comprising, a plug of sensitive primer composition adjacent to the point of the anvil and a ring of relatively insensitive composition surrounding the plug in adjacent relation.

5. A primer charge comprising a plug of sensitive primer composition centrally located, and a ring of relatively insensitive composition encircling the plug in adjacent relation.

6. A primer comprising, a sensitive increment of priming composition containing an initiator disposed to be acted upon by a detonating blow, and a relatively insensitive increment of the same ingredients as the first except that it is substantially devoid of initiator, said insensitive increment arranged to be ignited by the sensitive increment.

7. In the art of making primers the process comprising, suspending a priming composition containing an initiator in a vehicle, and dropping the suspension of initiator and vehicle into position in a priming cup.

8. In the art of making primers the process comprising, suspending a priming composition containing an initiator in a vehicle, dropping the suspension of initiator and vehicle into position in a priming cup, and covering the dropped suspension with a secondary mixture containing a fuel and an oxidizer.

9. In the art of making primers the process comprising, suspending a priming composition containing an initiator in a vehicle, dropping the suspension of initiator and vehicle into position in a priming cup, and covering the dropped suspension with a secondary mixture containing a waterproofing binder.

10. In the art of making primers the process comprising, fixing a sensitizer in the primer cup, covering the sensitizers with an initiator, and covering the initiator with a mixture containing a fuel and an oxidizer.

11. In the art of making primers the process comprising, fixing a sensitizers in the primer cup, covering the sensitizers with an initiator, and covering the initiator with a mixture containing a fuel and an oxidizer in a waterproofing binder.

12. In a primer having an anvil, a relatively small sensitive increment disposed adjacent the point of the anvil to be acted upon by a detonating blow and comprising an initiator, a fuel and an oxidizer, and a second increment disposed for ignition by the sensitive increment and containing a fuel and an oxidizing agent, said sensitive increment being so constituted as to produce the desired sensitivity characteristics of the primer and said second increment being so constituted as to produce the desired heat and flame characteristics of the primer.

13. In a primer having an anvil, a charge for the primer comprising initiator-containing-composition situated at the point of the anvil and disposed to be fired by the firing pin impact, and a fuel-oxidizer mixture relatively insensitive to impact or friction, disposed for ignition by the sensitive composition, said initiator-containing-composition being so constituted as to produce the desired sensitivity characteristics of the primer independently of said fuel-oxidizer mixture.

FREDERICK R. SEAVY.

65